

## UNITED STATES PATENT OFFICE

2,328,371

## LITHOGRAPHIC PLATE PREPARATION

William H. Wood, Bedford, Ohio, assignor to  
Harris-Seybold-Potter Company, Cleveland,  
Ohio, a corporation of Ohio

No Drawing. Application April 13, 1940,  
Serial No. 329,564

17 Claims. (CL 95—7)

In the manufacture of deep-etch lithographic plates it is customary to coat a cleaned and counter-etched zinc or aluminum plate with a "resist" which is sensitive to light, and the plate is then exposed to light in the form of the subject matter which is to be reproduced, such that in those areas where no image is desired on the finished plate the resist is hardened; then the unhardened areas of the resist are removed by a developing agent so as to leave the image portions of the plate clean. A so-called "deep-etching solution" is then applied to the plate and allowed to attack the exposed image areas until the metal is etched away to the desired depth, and after drying, the deep etched areas are treated with material, commonly referred to as a lacquer, to render them receptive to ink. Subsequently the light-hardened areas of the resist, which during etching have served to protect the non-image areas of the plate, are removed by a "clean-up" solution. The plate is then given a desensitizing etch to make the non-image areas receptive to water and is ready for printing. In accordance with the present invention, improved procedure and materials are involved, such as to afford more easy manipulation and control, and more reliable and positive action, and making possible the production of plates having improved longevity, definition, fidelity and uniformity.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

In the preparation of plates in accordance with my invention, I apply a combination of a water-soluble colloid coating material together with a material providing arabic acid. Illustrative of the water-soluble colloids are albumen, cold-water soluble gelatin, polyvinyl alcohol, dextrine, methyl-cellulose, etc. The action of arabic acid with these is to toughen them, thereby forming a peculiar toughened film. The arabic acid may be neutralized by a base and thereby yield a salt, increasing the solubility. Any base which produces a water-soluble salt of arabic acid is applicable. Illustrative of these are ammonium, sodium, potassium, organic bases, such as morpholine, ethanolamine, etc. The ammonium base is particularly desirable, being found to give an improved contrast between exposed and unex-

posed areas on the final plate, as compared with other bases. The arabic acid action in toughening, and the salt action in raising the solubility, afford thus two variable controls by which the amount of solubility and the amount of toughening respectively, may be directed as preferred in any given instance. Arabic acid is prepared by adding anhydrous alcohol to a solution of hydrochloric acid and gum arabic. Arabic acid is formed as a precipitate. This precipitate is washed several times with anhydrous alcohol, filtered and dried. It is then dissolved in water to form a solution of desired concentration, for example twenty per cent, and this solution is neutralized accurately with ammonium hydroxide, forming ammonium arabate. In using a "pH" meter, a pH of seven is desirable. The arabic acid compound is now combined with the water-soluble colloid, and for example this may involve one part of a twenty per cent water solution of egg albumen and four parts of a twenty per cent water solution of ammonium arabate. While these proportions are particularly desirable, up to equal amounts of the two solutions may advantageously be used.

Such combination material for coating, suitably sensitized with a soluble dichromate or the like as usual, is coated onto the metal plate, as by the usual means. This coating or resistant material gives certain notable new results and advantages: (1) it flows more readily and uniformly than the known gum or gum-glue solutions; (2) it forms a very thin coating while preserving its protective quality and thus minimizes the distortion of tone values which in known resists results from the spreading of the light during exposure; (3) the exposure required is relatively uninfluenced by the humidity of the surrounding air and in this respect is very much less effected than is the case with the usual resists; (4) it has special receptivity to action by the developer materials described hereinafter, in those areas which are unhardened by light, thus making possible an improved developing action over that which can be attained with the usual resists treated with known developers or treated with the new developer materials.

The coated metal plate (the metal being usual or as preferred, zinc, aluminum, etc.), having been exposed to light and the subject matter which is to be reproduced, is treated with the developer. Any developer as customary in the art may be employed, or preferably that in accordance with my patent application Serial No. 223,523, as this in conjunction with the present coating

gives outstanding advantages. This developer involves a solution of magnesium chloride and a hydroxydicarboxylic acid, such as malic acid, or somewhat less desirably tartaric acid. For example there may be 65 to 72 per cent <sup>5</sup>  $MgCl_2 \cdot 6H_2O$  and 2.5 to 5 per cent of the hydroxydicarboxylic acid.

Following removal of the unhardened portions of the coating or resist by the developer, the plate may be etched in customary or preferred procedure; and the hardened resist is next removed from the non-image areas of the plate which it has protected during the etching, and the plate is finished, as usual.

This application is a continuation, in part, as <sup>15</sup> to common subject matter, of my Patent No. 2,265,829, issued December 9, 1941.

Other modes of applying the principle of the invention may be employed, change being made as regards the details described, provided the <sup>20</sup> features stated in any of the following claims, or the equivalent of such, be employed.

I therefore particularly point out and distinctly claim as my invention:

1. In a process of making lithographic plates, applying to the plate a surfacing of ammonium arabate and egg albumen in the proportions of one part of a twenty per cent solution of albumen to one to four parts of a twenty per cent solution of the arabate, and providing a light-sensitizing agent. <sup>25</sup>

2. In a process of making lithographic plates, applying to the plate a surfacing of ammonium arabate and egg albumen, the proportion of the former in general not exceeding the latter, and at any desired stage providing a light-sensitizing agent. <sup>30</sup>

3. In a process of making lithographic plates, applying to the plate a surfacing of a water-soluble colloid other than gum arabic together with ammonium arabate, and at any desired stage providing a light-sensitizing agent. <sup>35</sup>

4. In a process of making lithographic plates, applying to the plate a surfacing of a water-soluble colloid other than gum arabic together with a material providing an arabic acid radical from the group consisting of arabic acid and salts formed by reacting arabic acid with a base, and at any desired stage providing a light-sensitizing agent. <sup>40</sup>

5. In a process of making lithographic plates, toughening a water-soluble colloid coating other than gum arabic by inclusion of arabic acid, and at any desired stage providing a light-sensitizing agent. <sup>45</sup>

6. In a process of making lithographic plates, applying to the plate a surfacing of a water-soluble colloid other than gum arabic and arabic acid with a base which produces a water-soluble salt of arabic acid, and at any desired stage providing a light-sensitizing agent. <sup>50</sup>

7. In a process of making lithographic plates, <sup>55</sup>

applying to the plate a surfacing of a water-soluble colloid other than gum arabic and arabic acid, and controlling the degree of solubility of the latter by inclusion of a base which produces a water-soluble salt of arabic acid, and at any desired stage providing a light-sensitizing agent. <sup>60</sup>

8. In a process of making lithographic plates, applying to the plate a surfacing of a water-soluble colloid other than gum arabic, and toughening the colloid by inclusion of arabic acid, and controlling the solubility of the arabic acid by inclusion of a base which produces a water-soluble salt of arabic acid, and at any desired stage providing a light-sensitizing agent. <sup>65</sup>

9. In a process of making lithographic plates, applying to the plate a surfacing of a water-soluble colloid other than gum arabic and arabic acid, and subsequently treating the surface with a solution of magnesium chloride and malic acid, and at any desired stage providing a light-sensitizing agent. <sup>70</sup>

10. In a process of making lithographic plates, applying to the plate a surfacing of a water-soluble colloid other than gum arabic and arabic acid, and subsequently treating the surface with a solution of magnesium chloride and a hydroxydicarboxylic acid, and at any desired stage providing a light-sensitizing agent. <sup>75</sup>

11. A lithographic plate surfaced with ammonium arabate and egg albumen, and at any desired stage provided with a light-sensitizing agent. <sup>80</sup>

12. A lithographic plate surfaced with the products of arabic acid and a water-soluble colloid other than gum arabic, and at any desired stage provided with a light-sensitizing agent. <sup>85</sup>

13. A lithographic plate surfaced with ammonium arabate and a water-soluble colloid other than gum arabic, and at any desired stage provided with a light-sensitizing agent. <sup>90</sup>

14. A lithographic plate surfaced with a water-soluble colloid other than gum arabic and a material providing an arabic acid radical from the group consisting of arabic acid and salts formed by reacting arabic acid with a base, and at any desired stage provided with a light-sensitizing agent. <sup>95</sup>

15. A lithographic plate surfaced with a water-soluble colloid other than gum arabic, and arabic acid and a salt of arabic acid, and at any desired stage provided with a light-sensitizing agent. <sup>100</sup>

16. In a process of making lithographic plates, applying to the plate an ammonia-neutralized aqueous solution of a precipitate from addition of alcohol to a hydrochloric acid solution of gum arabic. <sup>105</sup>

17. A lithographic plate having a surface formed from ammonia-neutralized aqueous solution of a precipitate from addition of alcohol to a hydrochloric acid solution of gum arabic. <sup>110</sup>

WILLIAM H. WOOD.